

Nov. 12, 1946.

F. T. POWERS

2,411,109

ETCHING ROTOGRAVURE PRINTING MEMBERS

Filed Feb. 26, 1944

Fig. 1



Fig. 3

Fig. 2



INVENTOR.  
Frank T. Powers  
BY  
Hobart N. Durham  
Attorney

## UNITED STATES PATENT OFFICE

2,411,109

ETCHING ROTOGRAVURE PRINTING  
MEMBERS

Frank T. Powers, Glen Cove, N. Y.

Application February 26, 1944, Serial No. 524,075

2 Claims. (Cl. 95—5.7)

1

The present invention relates to new and useful improvements in the preparation of rotary and intaglio printing members and particularly rotary photogravure cylinders.

Objects and advantages of the invention will be set forth in part hereinafter and in part will be obvious herefrom, or may be learned by practice with the invention, the same being realized and attained by means of the processes, steps and combinations pointed out in the appended claims.

The invention consists in the novel steps, processes, combinations and improvements herein shown and described.

The accompanying drawing, referred to herein and constituting a part hereof, illustrates one manner of carrying out the process of the invention, and together with the description, serves to explain the principles of the invention.

Of the drawing:

Figure 1 is a perspective view showing diagrammatically one step of the process of the present invention;

Figure 2 is a diagrammatic view, with certain parts exaggerated, showing a transparency applied to the surface of the coated cylinder for exposure of the resist prior to etching; and

Figure 3 is a diagram showing the method of exposing the cylinder resist beneath the transparency.

The present invention has for its object the provision of a novel and improved process of photoengraving, particularly for rotary, intaglio printing members. A further object is the provision of an improved process of preparing rotary photogravure cylinders. The invention further provides an improved process of coating a cylinder with photosensitive resist, exposing the resist and developing the resist so that it may be etched to provide a rotary photogravure printing cylinder.

In the conventional process of rotary photogravure, the ground and polished cylinder of copper is cleansed and on it is transferred a layer of exposed photosensitive gelatin which has been exposed to a continuous tone transparency of the picture to be reproduced, as well as a rotogravure screen, after which the layer is developed and etched in varying strengths of ferric chloride. However, such a process depends upon the transfer of a previously exposed layer of colloid, the precise and skilful development of the layer, and then the etching in selected strengths of etch, which not only etch the copper, but also wear away the gelatin film so as to etch the copper to varying depths in the various intagliated cells.

2

In accordance with the present invention, the copper cylinder is coated with a solution of gelatin and a bichromate to provide a thin, uniform layer of resist on the surface of the cylinder. Preferably warm bichromate gelatin solution is poured on the cylinder as it is rotated to form the uniform film, and the cylinder is revolved until dry, in a current of warm air, if desired. When dry, the layer is exposed through a combined screen and continuous tone transparency, preferably comprising the positive transparency print on strip film of a conventional halftone photoengraving negative which provides a uniform number of dots per unit area, which dots vary in size or area in accordance with the tones to be reproduced. This strip film transparency is wrapped around the coated cylinder in intimate contact therewith, preferably in page size areas, with the sheets held in place by scotch tape or otherwise until after exposure. When the cylinder has been completely covered by the transparencies, it is exposed in actinic light, preferably a longitudinally extending beam of light, as the cylinder is revolved to distribute the exposure uniformly. When sufficiently exposed, the transparency is removed, the cylinder developed in water considerably warmer than the body of the cylinder and when the cylinder has been completely developed, the cylinder is suitably etched, as for instance in an aqueous solution of ferric chloride. When fully etched, the remaining resist may be removed from the cylinder by means of an alkaline solution, such as dilute caustic soda, thereby rendering the cylinder ready for printing in the usual manner.

The printing member produced by the present invention is superior to the conventional rotogravure member, as the image on the printing member is formed of intagliated cellular cavities of substantially uniform depth which vary in area in accordance with the tone to be reproduced. Furthermore the etching is accomplished with much more certainty than is usual and depends in no way upon the humidity of the gelatin or ambient atmosphere.

It will be understood that the foregoing general description and the following detailed description as well are exemplary and explanatory of the invention but are not restrictive thereof.

Referring now in detail to the details of the preferred process according to the present invention, the steps of which are partially illustrated in the accompanying drawing, the member to be etched comprises a ground and polished cylinder 50 having a surface layer which is preferably a

substantial thickness of copper. As this cylinder is slowly rotated, it is coated with a photosensitive resist which preferably comprises a bichromated gelatin solution of substantially the following proportions:

|                         |       |      |
|-------------------------|-------|------|
| Water                   | cc.   | 4000 |
| Soft gelatin            | grams | 400  |
| Ammonium bichromate     | do    | 80   |
| Ferric ammonium citrate | do    | 80   |

This sensitized resist is slowly poured on the surface of the rotating cylinder to provide an excess of resist as the stream is moved from one end of the cylinder to the other, and rotation of the cylinder is continued until the resist has gelled and dried, preferably assisted by a current of warm air directed against the cylinder 10.

When the thin layer of resist 11 has dried, the cylinder is ready to receive the transparency for the photographic exposure. This transparency is preferably made from a conventional photoengraving halftone camera negative on paper strip film and is developed, fixed and washed in the usual manner. Alternatively, the transparency may be formed by making a halftone copy of a continuous tone negative of the desired copy through a halftone screen, (in the conventional manner of making a halftone negative except that a negative rather than positive copy is used). Thus in the shadows, the transparency comprises small transparent dots, while in the highlights, the transparency comprises large transparent dots which may merge to leave only small opaque dots.

After processing, the transparency comprises a thin flexible film 14 which when dry may be wrapped on the surface of the resist-coated cylinder 10 to bring it into intimate contact with the resist on the surface of the cylinder where it may be held by scotch tape 12 around the edges of each sheet of film, the several sheets of each conveniently being of page size.

With the several films assembled in proper position on the cylinder surface the resist is exposed to actinic light through the transparencies for a time sufficient to render it fully exposed. This exposure is preferably carried out by rotating the cylinder at a fairly slow rate adjacent to a light source 16 of actinic light extending longitudinally of the cylinder, such as a mercury vapor lamp which may be shielded by the opaque members 18. The rotating of the cylinder 10, continued for a considerable period of time, produces a uniform illumination of the transparencies 14 and resist layer 11.

After the exposure is complete, the transparencies 14 are removed and the cylinder 10, which is at room temperature of about 70° to 80° F., is

ready for development which may be carried out by spraying with, or rotation in water at 120° to 140° F., approximately. Alternatively, the resist may be developed in a 1% aqueous solution of a substantive dye such as brilliantbenzoecht-violet (Schultz 1931 Edition No. 610 BL, 2 RL). The resist may then be hardened by immersion for a few moments in a dilute solution 1% or 2% of a chromic acid compound or other hardening agent which reacts with the dye to harden the gelatin in accordance with the process of my co-pending application Serial No. 524,074, filed February 26, 1944.

After drying and rinsing with water, the cylinder may be etched by treatment with a suitable mordant such as aqueous ferric chloride in the usual manner of photoengraving, not requiring the varying strengths of mordant as is usual with rotogravure.

When the proper depth is attained, the cylinder 10 may be rinsed, dried and proved, after which the resist 11 may be stripped by means of a dilute alkaline solution.

The process is highly advantageous in connection with multicolor work, as the etching is much more readily controlled than usual, requires less hand work and the cylinders may be proved and if needing correction may be again etched before the resist is removed.

The invention in its broader aspects is not limited to the specific processes and steps shown and described but departures may be made therefrom within the scope of the accompanying claims without departing from the principles of the invention and without sacrificing its chief advantages.

What I claim is:

1. The process of photoengraving a cylinder which comprises coating the surface of the cylinder with a layer of photosensitive gelatin resist, exposing the resist to the desired image and developing the exposed resist by treatment with water substantially warmer than the body of the cylinder to wash away the not fully exposed gelatin resists, dyeing the resist with a substantive dye, and hardening the resist by a compound reactive with the dye.

2. The process of photoengraving a cylinder which comprises coating the surface of the cylinder with a layer of photosensitive gelatin resist, exposing the resist to the desired image and developing the exposed resist by treatment with water substantially warmer than the body of the cylinder to wash away the not fully exposed gelatin resists, dyeing the resist with a substantive dye, hardening the resist by a chromic acid solution, and etching the cylinder.

FRANK T. POWERS